

## UNITED STATES PATENT OFFICE

RHETHERFORD B. MARTIN, OF ROSELLE, NEW JERSEY, ASSIGNOR TO AMERICAN CYANAMID COMPANY, OF NEW YORK, N. Y., A CORPORATION OF MAINE

## MINERAL CONCENTRATION

No Drawing.

Application filed October 31, 1928. Serial No. 316,354.

This invention relates to the treatment of ores, and more particularly has reference to mineral collecting agents and the separation and concentration of valuable constituents from ores, and like bodies containing more than one mineral, by a flotation process.

Heretofore separation and concentration of valuable mineral constituents from ores by various methods have been carried out. All of those methods are more or less expensive, resulting in relatively high costs of production, especially when the ore treated is poor in the constituent sought.

One particular method heretofore employed has comprised the steps of grinding the ore to fine particles, and then subjecting the mass to a flotation process in which there is employed a frothing agent, such as pine oil or other substances capable of producing a froth.

Some organic compounds, particularly certain alkyl thiocarbonates, when introduced into a flotation process materially increase the efficiency thereof, resulting in a greater yield of the desired constituents under the same operating conditions or by accomplishing the same results with a smaller amount of material.

In spite of the remarkable properties of the alkyl thiocarbonates heretofore used, and the increased efficiency afforded by their use, flotation processes are not carried out in as efficient and economical a manner as is desirable and possible to attain.

An object of this invention is to devise a method of treating ores and like bodies to effect a separation and concentration of their valuable constituents that is more efficient than any other method heretofore practiced.

With this and other objects in view which may be incident to my improvements, the invention in general comprises the separation of minerals from their ores or associated

bodies by a flotation process, utilizing a suitable frothing medium together with an improved mineral collecting agent.

In carrying out my invention by the well known flotation process, I employ a suitable frothing agent or frothing aromatic sub-

stances such as cresylic acid, cresote and phenol. The ore is properly prepared by grinding, classifying, diluting, and with or without conditioning with other modifying agents.

After the ore is made up into a pulp suitable for the flotation process, and, at a desired time, a hydrogenated aromatic sulphur compound is introduced therein. This sulphur compound differs from the well known thioureas and alkyl thiocarbonates, in that it is formed from the interaction of hydrogenated phenols, carbon disulphide and a suitable alkali metal hydroxide such as sodium and potassium. Both frothing and collecting properties are possessed by the phenols, and on treatment with sulphur or inorganic sulphides these substances act to improve the flotation process.

It has been difficult to form beneficial flotation reagents by treating certain phenols with carbon disulphide and sodium hydroxide, for instance, dissolved in water. Hydrogenation of these hydrocarbons in the presence of a catalyst, such as nickel or other suitable substances, at temperatures between 180° and 250° C., produces hydrogen additive compounds. Moreover, by completely hydrogenating, for example, cresol, there is produced methyl cyclohexanol,  $\text{CH}_3\text{C}_6\text{H}_{10}\text{OH}$ .

I have discovered that methyl-cyclohexanol reacts readily with carbon disulphide and sodium hydroxide dissolve in water to form what I believe to be sodium methyl-cyclohexanyl xanthate, as indicated below:



The components entering into the reaction to form sodium methyl-cyclohexanyl xanthate are preferably in the following proportion:

| 4 mols. methyl-cyclohexanol                                                                                     | Per cent | 95   |
|-----------------------------------------------------------------------------------------------------------------|----------|------|
| $\text{C}_6\text{H}_{10}\text{CH}_3\text{OH}$                                                                   |          | 35.8 |
| 6 mols. carbon disulphide $\text{CS}_2$                                                                         |          | 35.9 |
| 9 mols. sodium hydroxide $\text{NaOH}$ (sodium hydroxide dissolved in half its weight of $\text{H}_2\text{O}$ ) |          | 28.3 |

This compound is prepared by dissolving 28.5 parts by weight of caustic soda (96% pure NaOH) in 14.3 parts by weight of distilled water and cooling the solution formed

5 to 25° C. This solution is placed in a suitable receptacle and while shaking the receptacle, or otherwise agitating the solution, 35.8 parts by weight of methyl-cyclohexanol and 35.9 parts by weight of carbon disulphide are 10 added all at once. A reaction takes place slowly and the reaction mixture gradually becomes a light straw-yellow color. The mixture should be well agitated and kept fairly cold at all times by any suitable method and 15 means of cooling.

After a sufficient time, generally not longer than an hour, the reaction mixture solidifies. Up to the time of solidification, there is not much rise in the temperature of the reaction 20 mixture, and the temperature does not rise to a dangerous point, even upon prolonged standing without cooling. All the while the reaction is taking place there is a gradual darkening in color and when the reaction is 25 finally completed, the mixture assumes a more or less dark brick red color.

The crude reaction mixture consists of some sodium carbonate together with sodium thiocarbonate, sodium sulphohydrate and the desired sodium methyl-cyclohexanyl xanthate. If it is desired to isolate the pure sodium methyl-cyclohexanyl xanthate, the crude reaction product can be extracted with acetone. After filtering, the acetone solution containing the sodium methyl-cyclohexanyl xanthate can be treated with ether to cause the sodium methyl cyclohexanyl xanthate to precipitate therefrom.

This new thiocarbonic acid derivative of 40 hydrogenated cresylic acid is soluble in water, alcohol, acetone, etc. It has a water cress odor and seems to decompose when heated to temperatures of from 90 to 110° C, with a darkening in color. It appears that this new compound is formed according to the following reaction equation:



50 It will be clear from the above reaction that the methyl-cyclohexanol reacts with the sodium hydroxide and carbon disulphide in a manner characteristic of alcohols.

55 If desired, the reaction product may be purified as described above, or by any other method, to secure pure sodium methyl-cyclohexanyl xanthate. When the compound is to be used as a mineral collecting agent it is not 60 necessary to purify the reaction product, since the by-products formed along with the sodium methyl-cyclohexanyl xanthate do not detrimentally affect the mineral collecting properties of the xanthate compound. The 65 crude reaction product which may be intro-

duced directly into the mineral flotation process without purification, contains approximately 70% of sodium methyl-cyclohexanyl xanthate.

While, for purposes of illustration, the type 70 xanthate compound has been described with reference to hydrogenated cresylic acid (methyl-cyclohexanol), I wish it to be clearly understood that the homologues and analogues of methyl-cyclohexanol can be used to 75 prepare xanthates having properties similar to sodium methyl-cyclohexanyl xanthate. Instead of using cresylic acid as the basic substance to be hydrogenated and finally converted into a xanthate, phenol may be hydro- 80 genated and employed as described and claimed in application Serial No. 292,607, filed July 13, 1928. Besides phenol, as listed below, any of the following substances can be advantageously utilized:

|           |    |
|-----------|----|
| Phenol    | 85 |
| o-Xylenol |    |
| p-Xylenol |    |
| Cumenol   |    |
| Carvacrol |    |
| Thymol    | 90 |
| Eugenol   |    |
| Orcinol   |    |

Besides being susceptible to variations in 95 the alcohols or alcoholic reacting substances entering into the reaction to form the xanthates, these compounds are also susceptible to variations in the metallic hydroxides entering into the reaction. For example, potassium hydroxide, and hydroxides of the other alkali metals may be employed to produce xanthates having properties very similar to the sodium compound described in detail above.

In carrying out the separation of minerals 100 in accordance with my invention, the ore is properly prepared by grinding, classification and dilution, and conditioning with other modifying agents if desired. The ore is then subjected to a flotation process employing a suitable frothing agent or frothing aromatic substance such as cresylic acid or other similarly reacting substances. After the above preparation, the sodium methyl-cyclohexanyl xanthate or other corresponding compound is 110 introduced into the ore pulp.

The following tabulation illustrates a test run on a sample:

|                                                     |                     |
|-----------------------------------------------------|---------------------|
| Utah Copper Mill heads, assaying 0.94% Cu.          | 120                 |
| Ground with 5 lbs. burnt lime per ton of ore        |                     |
| Sodium methyl-cyclohexanyl xanthate, as a collector | 0.04 lbs. per T.    |
| Cresylic acid, as a frothing agent                  | 0.1 lbs. per T. 125 |
| Copper concentrate                                  | 16.54% Cu.          |
| Copper tailings                                     | .05% Cu.            |
| Percentage extraction                               | 95%                 |

From the foregoing results, it will be appreciated that the new mineral collecting agents 130

forming the subject matter of this application, materially and advantageously affect mineral separation processes in which they are employed. Also, the compounds hereinbefore described may be rather easily prepared from relatively low cost raw materials which, together with the effectiveness of the compounds, results in low production costs of the mineral products.

10 These new flotation agents stabilize mineral flotation froth, have selective properties, drop iron from copper ores, are active collectors on zinc ores and are very effective even on coarsely ground ores. The latter is particularly desirable as much time can be saved in the preparation of the ores prior to treatment. Thus it will be seen that this invention makes it possible to more efficiently separate minerals from their ores than heretofore 20 accomplished.

While I have herein shown and described a practical and satisfactory process and agent for carrying out my invention, it is, of course, obvious that various modifications may be 25 made therein without exceeding the scope of my invention, it being understood, for example, that the homologues and analogues of the hydrogenated phenolic bodies may be employed in combination with carbon disulphide 30 and alkali metal hydroxides to produce flotation collecting agents.

I claim:

1. A method of froth flotation for ores and like bodies comprising introducing into a 35 suitably conditioned ore pulp a thiocarbonic acid derivative of a hydrogenated methyl compound of a cyclic hydrocarbon so as to concentrate the values.

2. A froth flotation method for concentrating ores and like bodies comprising introducing into an ore pulp a salt of a hydrogenated cresyl derivative of di-thiocarbonic acid so as to concentrate the value.

3. In a froth flotation method for concentrating ores and like bodies the step of introducing into an ore pulp a reagent formed from a methyl derivative of a hydrogenated phenol, carbon disulphide, sodium hydroxide and water.

4. In a froth flotation method of concentrating ores and like bodies the step of introducing into an ore pulp a thiocarbonic acid derivative of a hydrogenated methyl substituted phenol.

5. A froth flotation method for concentrating ores and like bodies comprising introducing into ore pulp a thiocarbonic acid derivative of hydrogenated cresol so as to concentrate the value.

6. A method of froth flotation for ores and like bodies comprising introducing into ore pulp an alkali metal salt of a thiocarbonic acid compound containing a methyl derivative of cyclohexanol so as to concentrate the value.

7. In a froth flotation method for concentrating ores and like bodies the step of introducing into ore pulp sodium methyl-cyclohex- 70 anyl xanthate.

8. A method for treating an ore comprising 75 grinding the ore into particles, classifying and conditioning the mass by adding a frothing agent thereto and introducing therein a thiocarbonic acid derivative of hydrogenated cresol.

9. In a flotation method for concentrating ores and like bodies, the step of introducing into an ore pulp, an alkali methyl cyclohex- 80 anol xanthate.

10. In a froth flotation method for concentrating ores, the step of introducing into an ore pulp, an alkali metal alkyl substituted hydroaromatic alcohol xanthate.

11. In a froth flotation method for concentrating ores, the step of introducing into 85 an ore pulp, an alkali metal alkyl substituted hydroaromatic monohydroxy alcohol xanthate.

12. In a froth flotation method for concentrating ores, the step of introducing into an 90 ore pulp, an alkali metal poly alkyl substituted hydroaromatic alcohol xanthate.

13. In a froth flotation method for concentrating ores, the step of introducing into an ore pulp, an alkali metal poly substituted 95 hydroaromatic alcohol xanthate.

In testimony whereof I affix my signature.

RHETHERFORD B. MARTIN.

100

105

110

115

120

125

130